# EUROPEAN PATENT SPECIFICATION

(11) **EP 3 122 475 B1**
(45) Date of publication and mention of the grant of the patent: **12.06.2019**
(21) Application number: 15713375.2
(22) Date of filing: 20.03.2015
(51) Int. Cl.: B05D 3/06, B05D 1/42, B05D 3/02, B05D 1/28

(54) **PROCESS FOR PAINTING FLAT SUBSTRATES HAVING HIGH SURFACE PERFECTION WITH RADICAL POLYMERIZATION INDUCED BY LED LAMPS AND THE ELEMENTS PAINTED WITH THIS PROCESS**
VERFAHREN ZUM LACKIEREN VON FLACHEN SUBSTRATEN MIT HOHER OBERFLÄCHENPERFEKTION MIT RADIKALISCHER POLYMERISATION DURCH LED-LAMPEN UND MIT DIESEM VERFAHREN LACKIERTE ELEMENTE
PROCÉDÉ POUR PEINDRE DES SUBSTRATS PLATS PRÉSENTANT UNE HAUTE PERFECTION DE SURFACE AVEC UNE POLYMÉRISATION RADICALAIRE INDUITE PAR LAMPES À DEL, ET ÉLÉMENTS PEINTS AU MOYEN DE CE PROCÉDÉ

(30) Priority: 26.03.2014 IT AN20140049
(43) Date of publication of application: 01.02.2017
(73) Proprietor: INDUSTRIA CHIMICA ADRIATICA - S.P.A. - in sigla ICA S.P.A., 62012 Civitanova Marche (MC) (IT)
(72) Inventor: SPARAPANI, Luca, I-62014 Petriolo (MC) (IT); PANICCIA, Fabio, I-62012 Civitanova Marche (MC) (IT)
(74) Representative: Statti, Francesco
(86) International application number: PCT/EP2015/000620
(87) International publication number: WO 2015/144304

(56) References cited:
- WO-A1-2013/123107
- WO-A2-02/068189

## Description

### Field of the Invention

The present invention concerns a process for finishing substrates made of plastic, laminated or wooden material, in particular polymethylmethacrylate (PMMA), between 10 micron and 1 cm thick, using paints with radical cross-linking induced by LED sources with wavelengths between 320 and 450 nm, and the elements obtained with this process.

### Background of the Invention

PMMA is a plastic material that has excellent mechanical and optical properties, such as excellent light stability and an intrinsic low resistance to chemical agents. But PMMA is not scratch resistant, although it has better resistance than other plastics.

For this reason, by applying a layer of protective paint on the surface of the PMMA, it is possible to improve its mechanical and chemical properties, leaving its optical properties unchanged.

For example, it is possible to use paints that will improve their surface hardness, chemical resistance, surface cleanliness, slipperiness and scratch-proof properties, provided that they are applied in such a way as to ensure their good adhesion to the painted substrate, their good level of polymerization and their high surface hardness.

To obtain these technical results more easily, paints with radical cross-linking induced by UV radiation are known (hereinafter called UV paints), characterized by rapid polymerization (milliseconds), high surface hardness and high degrees of cross-linking.

UV paints can be diluted with water, with solvent or be without either. These last, hereinafter called 100% UV paints, are the most suitable because, since they are without solvents and water, they have rapid polymerization times and other advantages such as higher hardness, higher scratch resistance and low degree of yellowing on exposure to natural elements.

100% UV paints are generally mixtures of copolymers containing unsaturated bonds and the presence of one or more acrylic or polyester groups with acrylic monomers and photoinitiators. Moreover, these paints can be mixed with silicone substances, polysiloxanes, waxes or other substances to improve some properties such as slipperiness, spreading, wetting of the substrate, adhesion or other surface characteristics.

Solvent-based UV paints are generally made as above, but solvent is added to aid their spreading, ease of application and adhesion to the substrate, if it is necessary to improve these characteristics compared to 100% UV paints.

But water-based UV paints are characterized by the use of water-thinnable copolymers, or by dispersions or aqueous emulsions of acrylic, polyurethane, urethane acrylate or polyester oligomers.

UV paint can be applied by spraying, by curtain coating, or by roller; the most suitable method is, however, by roller, due to its high speeds (up to 30 m/min) and also because it requires low quantities of paint (5-10 micron of paint) to be evenly applied over the entire surface to be painted, without using solvents and, above all, with a near 100% coefficient of transfer.

The problem with applying UV paint by roller is that a good spread of it over the painted surface is not obtained, so nullifying its aesthetic result and therefore altering the visual perception that can be obtained with PMMA.

To obviate this problem, known in the state of the art are patents US6423167B1 and US8191500B2 whose teaching has consisted of using a thin plastic material (hereinafter called *release*) to be spread over the painted surface so as to make distribution of the paint even and obtain a perfectly smooth surface.

The release is generally made of polyester (known by the commercial name of Mylar®, Melinex®, Lumirrot®, Terphane®, Hostaphane®), polypropylene, nylon, PET, PVF, CPP, silicone or any other thin (less than 1 cm) plastic material that is optically transparent or semi-transparent and with high transmittance at wavelengths below 380 nm.

The process of UV painting and treatment with release is generally called embossing. This process is currently used for the treatment of numerous flat surfaces, including wood - as per teaching of patent US20040094262A1; wood fibre as per teaching of patent EP2271492A2; laminates as per teaching of patent US6423167B1; glass, plastic. The treatment can give the surface to be painted a smooth or textured appearance, as per teaching of patent DE202004018710U1, so as to be able to control its gloss; or particular optical structures as per teaching of patent US20110011390A1.

UV paint is currently polymerized through the use of gallium or mercury doped UV lamps with powers between 80 W/cm and 200 W/cm. These lamps have variable emission, as shown in the graph of Fig. 1.

Normally, mercury lamps have an emission maximum at 320 and 360 nm and gallium lamps at 360 and 420 nm.

Patent US20100258051A1 describes and claims an *embossing* process in which UV paint is applied by roller; the release is applied immediately after the paint has been spread on, and the painted substrate, coupled with the release, is passed under one or more UV lamps to start the polymerization process. After passing under the UV lamp, the release is removed and then recovered.

The use of UV lamps poses numerous problems also connected with the optical properties of the release.

The first problem arises from the use of releases that are not completely transparent to UV radiation; in particular, there can be transmittance values below 5% for wavelengths below 320 nm. This causes the problem that photoinitiators, such as a-hydroxyketones and benzophenones, are poorly effective in the polymerization of the UV paints used, because these molecules have absorption maximums below 320 nm, with the consequence of having a low cross-linking density of the UV paint, low chemical resistance and low scratch and abrasion resistance, as well as adhesion problems and a marked yellowing of the paint on exposure to natural elements.

Moreover, there can be poor adhesion due to the low polymerization of the interface layer between the substrate and the paint.

These problems are even more evident if the paint has been applied on plastic substrates, where it is necessary to apply paint with high performance characteristics (called *hardcoat*) that will give protection to the painted substrate.

Another problem in the known UV paint application processes arises from the fact that UV lamps emit their energy only partially in the form of UV radiation, while most of the energy is emitted as visible light and high heat on the surface to be polymerized generated by parabolas.

The high heat is a problem in the process of painting plastic because it softens it, changes its surface structure and releases molecules that are not perfectly polymerized (elasticizers, phthalates, monomers, etc.) that can affect the paint polymerization process and the final properties of the paint.

UV radiation is generally an electromagnetic radiation between 4 and 380 nm *(*The American Heritage Dictionary of the English Language, Fourth Editi*on*).

To obviate this problem, alternative sources of UV radiation to the conventional arc lamps used up to now have been developed. These include LED lamps or sources (hereinafter called LED lamps), which can emit a monochromatic source of light at a specific wavelength. LED lamps can have powers between 2 and 20 W/cm and wavelengths between 300 and 420 nm. The most interesting, due to their characteristics of coupling with some photoinitiators for UV paints and due to their emission power, are LED lamps at 395 nm and at 365 nm, as shown in Fig. 2. These LED lamp wavelengths absorb photoinitiators such as acylphosphine oxides (BAPO, MAPO, TPO-L). This type of photoinitiator is widely used for making pigmented or thickly applied UV paints.

The use of a release, as well as improving the spreading of the UV paint, also has an inactivating function on the surface of the painted substrate. In fact, due to the contact between the release and the UV paint, the quantity of oxygen on the painted substrate is very low. This allows the problem of inhibition of the oxygen typically present in the polymerization of UV paints with LED lamps, due to the absence of UV radiation below 300 nm, to be overcome.

After polymerization, the release is removed from the surface of the painted substrate and is recovered.

The process of heating the surface of the substrate to be painted is particularly suitable if it is made of plastic because it aids its process of adhesion to the paint. In particular, as regards the PMMA substrate, between 10 micron and 1 cm thick, to be painted, it is necessary to pre-heat it to a temperature between 40 and 70°C at the time of contact with the paint. Lower temperatures can cause problems of adhesion of the paint on the PMMA substrate to be painted. Moreover, the temperature also aids the mechanism of spreading of the paint over the PMMA substrate to be painted. Heating can be carried out for example with IR, NIR, UV lamps, heating elements or any other equipment suitable for transferring energy in the form of heat.

The use of monochromatic LED lamps also provides undoubted advantages on the life of the release used. The radiation generated by a conventional UV lamp covers a wide spectrum of frequencies that range from UV to IR; this can trigger degradation mechanisms on the material used for the release that, over time, can change some chemical and physical properties (elasticity, transparency, etc.). This problem is even more evident with re-usable releases, or with continuous silicone releases. In particular, in continuous silicone releases, it is possible to observe a rapid decline in transparency due to the use of gallium UV lamps that trigger secondary mechanisms of degradation of the belt.

The use of a monochromatic LED lamp avoids this phenomenon, due to the absence of secondary interactions arising from undesired radiations, so ensuring much longer lifetimes for the release and therefore better performance over time.

The use of LED lamps for the polymerization of paints has been known for some time (for example, US 20130224495 A1, US 8569393 B2) as also has the use of acylphosphine oxide based photoinitiators for their polymerization (for example, EP2448427A). The use of inert atmospheres for the polymerization of UV paints is also a known process, but the most commonly used method is to use inert gases to remove oxygen from the surface of the paint to be polymerized (for example, US 8567936 B2).

The use of a single UV lamp or source for the complete polymerization of UV paint through a release is also a known process (for example, DE 102006053662 A1 or WO 1999061168 A1, WO 2002068189 A2), but in these patents the use of generic UV sources is mentioned, and no mention is made of monochromatic LED sources. However, in the above-mentioned example DE 102006053662 A1, the fact is mentioned that the release exerts an inactivating function to remove oxygen from the surface of the paint.

In the graph of Fig. 3, which shows the emission spectrum comparison between mercury lamp and 365 and 395 nm LED lamp, the typical transmittance of a continuous silicone belt and of a Mylar release are shown. It is evident how these releases partially or completely screen some wavelengths. In particular, it is clear how no UV radiation passes through below 320 nm, therefore making ineffective the use of many a-hydroxyketones as photoinitiators.

The use of LED lamps or sources with wavelengths above 320 nm therefore allows this problem to be overcome, by providing higher powers (expressed as W/cm²) than conventional arc lamps, with all the above-described benefits in terms of release life, lower generation of heat and a better degree of polymerization of the UV paint used.

### Disclosure of the Invention

It is an object of the present invention to solve the above-mentioned problems, by proposing a process for painting flat substrates made of plastic material, in particular polymethylmethacrylate (PMMA), between 10 micron and 1 cm thick, or of laminated or wooden material, based on paints with radical polymerization induced by LED lamps or sources.

It is another object of the present invention to obtain flat surfaces made of plastic material, in particular polymethylmethacrylate (PMMA), between 10 micron and 1 cm thick, or of laminated or wooden material, based on paints with radical polymerization induced by LED lamps, having high chemical and physical performance and high optical quality.

It is another object of the present invention to obtain the polymerization of paint without using conventional arc lamps.

It is another object of the present invention to have considerable advantages in the process of polymerization of paint in terms of:
- less heating of the substrate to be painted;
- higher emitted energy both as J/cm² and as W/cm²;
- better degree of cross-linking that means better chemical resistance and resistance to abrasion and scratching;
- less yellowing (*photobleaching*);
- reduction of residual emissions;
- lower energy consumption;
- no ozone generation;
- better stability over time of the LED lamp and longer life than conventional UV lamps.

It is a further object of the present invention to also include the elements painted with this method, consisting of flat substrates made of plastic material, in particular polymethylmethacrylate (PMMA), between 10 micron and 1 cm thick, or of laminated or wooden material, based on paints with high hardness and with high degree of cross-linking.

These and other objects are achieved with the present invention that concerns a process for painting substrates made of plastic material, in particular polymethylmethacrylate (PMMA), between 10 micron and 1 cm thick, or of laminated or wooden material, through the use of paints with radical cross-linking induced by LED sources with wavelengths between 320 and 450 nm with a variable power between 2 and 20 W/cm and the elements painted with this process.

Further features and advantages of the invention will be more readily apparent from the description of a preferred, but not exclusive, embodiment of the process that is the subject of the present patent application, illustrated by way of non-limiting example in the drawings, in which:
- Fig. 1 shows the emission spectra in power of gallium or mercury doped UV lamps;
- Fig. 2 shows the emission spectra in intensity of mercury lamps, LED lamps with wavelength of 365 nm and LED lamps with wavelength of 395 nm;
- Fig. 3 shows the emission spectrum comparison between mercury lamp and 365 and 395 nm LED lamp and also shows the transmittance of a continuous silicone belt and of a Mylar release;
- Fig. 4, Fig. 4a and Fig. 5 show the system for painting on the flat of these substrates in which the continuous flat substrate to be painted (not shown), for example reels of plastic, coincides in the figures with the conveyor belt (1); if the flat substrate to be painted is not continuous, for example slabs or panels, a suitable conveying method must be used, represented by elements (1) and (12).

### Detailed Description of the Invention

The present invention concerns a process for painting on the flat of substrates made of plastic material, in particular polymethylmethacrylate (PMMA), between 10 micron and 1 cm thick, or of laminated or wooden material, having a different conveying system depending on whether the substrate to be painted is continuous or non-continuous. When the substrate to be painted is continuous (on a reel), a continuous or non-continuous release and a conveyor belt (1) that coincides with the reel itself are used; whereas when the substrate to be painted is non-continuous (plastic slabs, wood or laminated panels), a non-continuous or continuous release and the conveyor belt shown in Fig. 4 with (1) and (12) are used.

The release is considered continuous when both element (9) and element (13) are present; it is considered non-continuous when element (9) is present and element (13) is absent.

There are therefore two types of substrate to be painted:
- discontinuous substrates, such as flat panelling;
- continuous substrates, such as reels of plastic or wooden material.

In the case of flat panelling, the conveying system consists of a conveyor belt (1) whose function is to bring the substrate into contact with the painting elements and the equipment connected with it, such as for example, the painting roller and the release. In the system with panelling, conveyor belt (12) is present and is a continuous system with conveyor belt (1).

If the substrate to be painted is on a reel, the conveyor belt (12) is not necessary, but it is necessary to use an unwinding (10) and winding (11) mechanism so as to move the substrate to be painted and keep it at the right tension to obtain an even painting of it and correct coupling of the release on the surface. The conveyor belt (12) can in any case be present, since it does not hinder the painting process.

In the case of reels, the conveying system consists of a reel unwinding mechanism (10) and a reel winding mechanism (11). The speed of the winding and unwinding mechanisms must be identical; the speed of these elements determines the speed of the conveying system. In this case too, the conveying system is used to bring the substrate into contact with the painting elements and the equipment connected with it, such as for example, the painting roller and the release.

In the system with reels, the element indicated in the figures with number (12) is not present and that is why it is represented with a broken line.

The conveying system for continuous or non-continuous substrates is at variable speed between 1 and 30 m/min.

The process for painting substrates made of plastic material, in particular polymethylmethacrylate (PMMA), between 10 micron and 1 cm thick, or of laminated or wooden material, that is the subject of the present invention is characterized in that it uses paints with radical cross-linking induced by one or more LED sources (6) with wavelengths between 320 and 450 nm with a variable power between 2 and 20 W/cm and this LED source (6) is placed at a height from the substrate to be painted of between 0.1 mm and 10 cm behind the release.

Before application of the paint, the surface of the flat substrate to be painted is cleaned of any residues with ionizing radiations or other cleaning systems; then the surface of the flat substrate is heated by heating elements, IR lamps, NIR lamps, or the use of plasma ionization technologies, corona treatment, and a combination of these to aid adhesion of the paint to the substrate to be painted.

In particular, as regards the PMMA substrate, between 10 micron and 1 cm thick, to be painted, it is necessary to bring it to a temperature between 40 and 70°C at the time of contact with the paint to aid its spreading and adhesion. Besides the surface made of PMMA, between 10 micron and 1 cm thick, polycarbonate, cellulose propionate or cellulose acetate, the substrate to be painted can alternatively also consist of wooden, plastic or cellulosic material, glass or combinations with each other.

Once the flat substrate to be painted has been placed on the conveyor belt (1) or (1, 12), paint is applied on it by a system of application rollers (2) and (3) each having a doctor roller (2a) (3a) with independent speed for regulating the quantity of paint to be applied. The application rollers (2) and (3) are coated with rubber or silicone or polyurethane or alternatively have a smooth surface engraved with regular structures (lines, dots or patterns). The system of application rollers (2) and (3), as described above and shown in Fig. 4, can be replaced by other paint application systems such as for example curtain coating, spray, *offset*, *flexo* or *slot-die* systems, mentioned only as alternatives but not described and not shown in the present application.

The quantity of paint to be applied on the flat substrate up to roller (5) can range between 2 and 100 micron. The function of roller (5) is also to couple the continuous painted flat substrate with the continuous or non-continuous release of known thickness or the non-continuous painted flat substrate with the non-continuous or continuous release of known thickness, on which the paint is evenly distributed for the distance between the coupling roller (5) and its recovery roller (8); moreover, one or more LED lamps or sources (6) for polymerization of the paint are positioned between the coupling roller (5) and the recovery roller (8). If the release is continuous, its movement is brought about by a system of upper winders (4) and (7) connected with the lower coupling roller (5) and recovery roller (8), as illustrated in Fig. 4a.

The painted flat substrate is ready to be protected with a peelable paint or with a protective coating of plastic material, or rewound by the winding mechanism (11).

The UV paint used can be free of volatile substances (100% paint) or contain water (water-based paint), or contain solvents (solvent-based paint).

In the first case, the UV paint is a mixture of oligomeric polymers, monomers, photoinitiators, additives, mineral fillers, pigments and dyes with a solid content above 30%.

In the second case, the 100% UV paint is a mixture of oligomeric polymers, monomers, photoinitiators, additives, mineral fillers, pigments and dyes with a solid content above 30% and containing water or solvents.

An example of formulation of a UV paint is the following:

| **Raw material** | **% by weight** |
|---|---|
| Aliphatic urethane acrylate oligomer | 40-50% |
| Acrylic monomer | 30-50% |
| Adhesion promoting additive | 0.5-5% |
| Photoinitiator | 1-5% |
| Additives | 0.1-2% |

An example of formulation for a solvent-based UV paint is the following:

| **Raw material** | **% by weight** |
|---|---|
| Aliphatic urethane acrylate oligomer | 80-20 % |
| Acrylic monomer | 10-70 % |
| Solvent | 5-70 % |
| Photoinitiator | 1-5 % |
| Additives | 0.1-2% |

An example of formulation for a water-based UV paint is the following:

| **Raw material** | **% by weight** |
|---|---|
| Water-based UV oligomer (dispersion, emulsion, solution) | 20-80 % |
| Water | 10-70 % |
| Additives | 0.1-5% |
| Photo initiator | 1-5 % |

The indicated formulation is applied by EPDM 40 shore roller with a quantity of 8 g/m². Prior to application, the substrate is subjected to a corona treatment and the surface is heated to 50°C.

Straight after application, or in any case within a few seconds, the release is applied on the painted surface (Melinex 425) and, after 10 seconds, the paint is polymerized with a LED lamp of 395 nm wavelength with power of 8 W/cm placed at 1 mm from the surface.

If it is necessary to use a UV paint containing solvent, the solvent must be removed from the film of paint applied on the substrate to be painted before application of the continuous or non-continuous release. This stage can take place by increasing the time, between 10 seconds and 10 minutes, between the stage of applying the paint on the substrate to be painted and the stage of contact with the coupling roller (5) of the release. During this stage, to aid the solvent evaporation process, it is possible to use hot air, IR lamps, laminar air flows, catalytic plates, or any other technology suitable for this application, also in combination with each other (14).

In this type of UV paint, the solvent content is generally between 10 and 70%. The process described above for products containing solvents must be adopted in the case of UV paints containing water, in which, as an alternative, it is possible to use the above-mentioned example formulation, using, in place of the aliphatic urethane acrylate oligomer, aqueous emulsions or aqueous solutions or aqueous dispersions of acrylic, polyurethane, urethane acrylate or polyester resins, or combinations of these.

Generally, the water content is between 10 and 70%.

For solvent-based and water-based UV paints, all the other application and polymerization conditions relevant to the type of release used remain unchanged.

Since the application of solvent-based or water-based UV paints on a surface of substrates made of plastic material, in particular polymethylmethacrylate (PMMA), between 10 micron and 1 cm thick, or of laminated or wooden material, requires more time for evaporation of the water or solvent from the applied film, Fig. 5 illustrates the variant of the above-described process, in which the painting line has been lengthened and a heating unit (14) having IR lamps, or heating plates, or hot air flows, or catalytic plates or whatever located before the coupling roller (5), has been added.

## Claims

1. Process for painting on the flat of substrates made of plastic material, in particular polymethylmethacrylate (PMMA), between 10 micron and 1 cm thick, or of laminated or wooden material, having a conveying system with variable speed between 1 and 30 m/min for flat substrates using a release made of plastic material according to known thicknesses, **characterized in that** it uses paints with radical cross-linking induced by one or more LED sources (6) placed at a height from the substrate to be painted of between 0.1 mm and 10 cm behind the release and having wavelengths between 320 and 450 nm and a variable power between 2 and 20 W/cm.

2. Process for painting on the flat of substrates made of plastic, laminated or wooden materials as claimed in claim 1 **characterized in that** the PMMA substrate to be painted is previously treated with ionizing radiations or other cleaning systems, also in combination with each other.

3. Process for painting on the flat of substrates made of plastic, laminated or wooden materials as claimed in claim 1 **characterized in that** the PMMA substrate to be painted must be brought to a temperature between 40 and 70°C at the time of its contact with the paint.

4. Process for painting on the flat of substrates made of plastic, laminated or wooden materials as claimed in claim 1 **characterized in that** the paint is applied by one or more rollers, one or more sprayers, one or more curtain coaters, one or more *slot-dies* or combinations with each other.

5. Process for painting on the flat of substrates made of plastic, laminated or wooden materials as claimed in claim 1 **characterized in that** the UV paint is a mixture of oligomeric polymers, monomers, photoinitiators, additives, mineral fillers, pigments and dyes with a solid content above 30%.

6. Process for painting on the flat of substrates made of plastic, laminated or wooden materials as claimed in claim 1 **characterized in that** the UV paint is a mixture of oligomeric polymers, monomers, photoinitiators, additives, mineral fillers, pigments and dyes with a solid content above 30% containing water or solvent.

7. Process for painting on the flat of substrates made of plastic, laminated or wooden materials according to claims 1, 6 **characterized by** a lengthening of the painting line and by a heating unit (14) having IR lamps, or heating plates, or hot air flows, or catalytic plates or whatever, located before the coupling roller (5) in the case of water-based UV paints or solvent-based UV paints.

8. Process for painting on the flat of substrates made of plastic, laminated or wooden materials according to the previous claims **characterized in that**, as well as consisting of a surface made of PMMA, polycarbonate, cellulose propionate or cellulose acetate, the substrate to be painted alternatively consists of wooden, plastic, cellulosic material, glass or combinations with each other.

## Patentansprüche

1. Verfahren zum flächigen Lackieren von Substraten aus Kunststoff, insbesondere Polymethylmethacrylat (PMMA) mit einer Stärke zwischen 10 µm und 1 cm, oder aus Schicht- oder Holzwerkstoff mit einem Fördersystem mit variabler Geschwindigkeit zwischen 1 und 30 m/Min. für flache Substrate unter Verwendung einer Freisetzung aus Kunststoff entsprechend besagter Stärken, **dadurch gekennzeichnet, dass** es Lacke mit radikaler Vernetzung verwendet, die durch eine oder mehrere LED-Quellen (6) induziert werden, die in einer Höhe von dem zu lackierenden Substrat zwischen 0,1 mm und 10 cm hinter der Freisetzung und mit Wellenlängen zwischen 320 und 450 nm und einer variablen Leistung zwischen 2 und 20 W/cm angeordnet sind.

2. Verfahren zum flächigen Lackieren von Substraten aus Kunststoff-, Verbund- oder Holzwerkstoffen nach Anspruch 1, **dadurch gekennzeichnet, dass** das zu lackierende PMMA-Substrat zuvor mit ionisierenden Strahlungen oder anderen Reinigungssystemen, auch in Kombination miteinander behandelt wird.

3. Verfahren zum flächigen Lackieren von Substraten aus Kunststoff, Verbund- oder Holzwerkstoffen nach Anspruch 1, **dadurch gekennzeichnet, dass** das zu lackierende PMMA-Substrat beim Kontakt mit der Farbe auf eine Temperatur zwischen 40 und 70 °C gebracht werden muss.

4. Verfahren zum flächigen Lackieren von Substraten aus Kunststoff, Verbund- oder Holzwerkstoffen nach Anspruch 1, **dadurch gekennzeichnet, dass** die Farbe mit einer oder mehreren Walzen, Sprühgeräten, Vorhangbeschichtungen, *Schlitzdüsen-Beschichtungen* oder Kombinationen miteinander aufgetragen wird.

5. Verfahren zum flächigen Lackieren von Substraten aus Kunststoff-, Verbund- oder Holzwerkstoffen nach Anspruch 1, **dadurch gekennzeichnet, dass** die UV-Farbe eine Mischung aus oligomeren Polymeren, Monomeren, Fotoinitiatoren, Additiven, mineralischen Füllstoffen, Pigmenten und Farbstoffen mit einem Feststoffgehalt von über 30 % ist.

6. Verfahren zum flächigen Lackieren von Substraten aus Kunststoff-, Verbund- oder Holzwerkstoffen nach Anspruch 1, **dadurch gekennzeichnet, dass** die UV-Farbe eine Mischung aus oligomeren Polymeren, Monomeren, Fotoinitiatoren, Additiven, mineralischen Füllstoffen, Pigmenten und Farbstoffen mit einem Feststoffgehalt von über 30 % ist, die Wasser oder Lösungsmittel enthält.

7. Verfahren zum flächigen Lackieren von Substraten aus Kunststoff, Verbund- oder Holzwerkstoffen nach den Ansprüchen 1 bis 6, **gekennzeichnet durch** eine Verlängerung der Lackierlinie und durch eine Heizeinheit (14) mit IR-Lampen, Heizplatten, Heißluftströmungen oder katalytischen Platten oder alles weitere, die bei wasserbasierten UV-Lacken oder lösemittelhaltigen UV-Lacken vor der Kupplungswalze (5) angeordnet ist.

8. Verfahren zum flächigen Lackieren von Substraten aus Kunststoff, Verbund- oder Holzwerkstoffen nach den vorstehenden Ansprüchen, **dadurch gekennzeichnet, dass** das zu lackierende Substrat neben einer Oberfläche aus PMMA, Polycarbonat, Cellulosepropionat oder Celluloseacetat alternativ aus Holz, Kunststoff, Cellulosematerial, Glas oder Kombinationen miteinander besteht.

## Revendications

1. Procédé permettant de peindre sur la surface plane de substrats en matière plastique notamment en polyméthacrylate de méthyle (PMMA) -, d'une épaisseur comprise entre 10 microns et 1 cm, ou encore en matériau stratifié ou en bois, qui dispose d'un système de convoyage dont la vitesse varie de 1 à 30 m/min pour les substrats plats utilisant un diffuseur en matière plastique en fonction d'épaisseurs connues, **caractérisé en ce qu'**il utilise des peintures à réticulation radicalaire induites par une ou plusieurs sources DEL (6) placées à une hauteur, par rapport au substrat à peindre, se situant entre 0,1 mm et 10 cm derrière le diffuseur et dont les longueurs d'onde sont comprises entre 320 et 450 nm, ainsi qu'une puissance variable allant de 2 à 20 W/cm.

2. Procédé permettant de peindre sur la surface plane de substrats en matière plastique, en matériau stratifié ou en bois selon la revendication 1, **caractérisé en ce que** le substrat en PMMA à peindre est préalablement traité par des rayonnements ionisants ou d'autres systèmes de nettoyage, mais également par combinaison entre ces systèmes.

3. Procédé permettant de peindre sur la surface plane de substrats en matière plastique, en matériau stratifié ou en bois selon la revendication 1, **caractérisé en ce que** le substrat en PMMA à peindre doit être porté à une température se situant entre 40 et 70°C au moment de son contact avec la peinture.

4. Procédé permettant de peindre sur la surface plane de substrats en matière plastique, en matériau stratifié ou en bois selon la revendication 1, **caractérisé en ce que** la peinture est appliquée par un ou plusieurs rouleaux, un ou plusieurs pulvérisateurs, une ou plusieurs coucheuses à nappe, une ou plusieurs filières à fente ou par combinaison entre ces systèmes.

5. Procédé permettant de peindre sur la surface plane de substrats en matière plastique, en matériau stratifié ou en bois selon la revendication 1, **caractérisé en ce que** la peinture UV est un mélange de polymères oligomères, de monomères, de photo-initiateurs, d'additifs, de charges minérales, de pigments et de colorants, avec une teneur en solides supérieure à 30 %.

6. Procédé permettant de peindre sur la surface plane de substrats en matière plastique, en matériau stratifié ou en bois selon la revendication 1, **caractérisé en ce que** la peinture UV est un mélange de polymères oligomères, de monomères, de photo-initiateurs, d'additifs, de charges minérales, de pigments et de colorants, avec une teneur en solides supérieure à 30 % contenant de l'eau ou un solvant.

7. Procédé permettant de peindre sur la surface plane de substrats en matière plastique, en matériau stratifié ou en bois selon les revendications 1 à 6, **caractérisé par** une extension de la ligne de peinture et par un corps de chauffe (14) doté de lampes infrarouges, de plaques chauffantes, de flux d'air chaud, de plaques catalytiques ou de tout autre système, situé avant le rouleau de couplage (5) en cas de peintures UV à base d'eau ou de peintures UV à base de solvant.

8. Procédé permettant de peindre sur la surface plane de substrats en matière plastique, en matériau stratifié ou en bois selon l'une quelconque des revendications précédentes, **caractérisé en ce que** le substrat à peindre, tout comme il est constitué d'une surface en PMMA, en polycarbonate, en propionate de cellulose ou en acétate de cellulose, peut être constitué par ailleurs d'un matériau en verre, en cellulose, en plastique, en bois ou de ces matériaux combinés.
